

H. ELDIDGE.  
PROCESS OF MAKING METALLIC ALLOYS.  
APPLICATION FILED DEC. 22, 1916.

1,246,571.

Patented Nov. 13, 1917.

Fig. 1.



Fig. 2.



Inventor.

Hillary Eldridge, per  
Thomas S. Crane, Atty.

# UNITED STATES PATENT OFFICE.

HILLIARY ELDRIDGE, OF NEW YORK, N. Y.

## PROCESS OF MAKING METALLIC ALLOYS.

1,246,571.

Specification of Letters Patent.

Patented Nov. 13, 1917.

Continuation of application Serial No. 83,751, filed March 13, 1916. This application filed December 22, 1916. Serial No. 138,362.

To all whom it may concern:

Be it known that I, HILLIARY ELDRIDGE, a citizen of the United States, residing at 645 Eighth avenue, New York, county of 5 New York, and State of New York, have invented certain new and useful Improvements in Processes of Making Metallic Alloys, fully described and represented in the following specification and the accompanying drawings, forming a part of the 10 same.

The present invention consists of a process for making alloys of metal by heating the less fusible metal to an alloying temperature, and subjecting such heated metal 15 to the vapor of a more fusible metal and effecting a complete union of the metals in a molten state.

This application is a continuation of my 20 application No. 83,751 filed March 13, 1916, and allowed August 16, 1916, being a substitute therefor, and claims the same subject-matter as that allowed application.

Such alloys can be formed at a temperature 25 below the melting temperature of the less fusible metal, and the process can therefore be effected by heating the less fusible metal to an alloying temperature without melting it, or it may be effected by 30 melting the less fusible metal.

The process is especially applicable to the manufacture of any alloy of copper with such metals as zinc, antimony, lead, tin, or other volatile metals which melt and volatilize at a relatively low temperature, and are therefore liable to material loss by volatilization if the alloying metal be melted 35 with the copper in an open vessel.

In this process, the vapor of the alloying 40 metal is brought into direct contact with the heated copper and is absorbed by the copper whether in a melted state or merely heated to a suitable temperature, the alloy thus formed running off from the surface 45 of the copper, if solid, and exposing a new surface to a continuation of the same action.

If the copper be melted, the vapor of the alloying metal may be blown or forced 50 through the melted copper, to be absorbed by the copper, if the mass of the metals be considerable.

The use of the vapor effects a more thorough and gradual formation of the alloy than the mere melting of the metals together.

One great advantage of the invention is that the vapor of the more fusible metal can be procured directly from an oxid or ore of the alloying metal, the alloy being thus obtained much more advantageously 60 than if made with the metal itself.

When procuring the zinc vapor from an oxid or ore of that metal, a reducing agent, as carbon in any convenient form, is mixed with the oxid or ore and placed in the receptacle containing the metal thereby maintaining a reducing atmosphere which has the further effect of purifying the alloy by reducing such oxides as it may contain.

The zinc vapor can be derived from any 70 ore of zinc which with a suitable reagent may, under the influence of heat, be reduced to an oxid of the metal; as for example, a sulfate, a carbonate, &c. The use of such an ore or oxid of zinc is much less costly 75 than the use of metallic zinc.

In the drawing, Figure 1 is a diagram in vertical section of a furnace for heating a crucible; and Fig. 2 is a diagram in vertical section of a furnace with two connecting 80 chambers.

An apparatus is shown in the annexed drawing for heating a crucible containing all the ingredients, having a furnace-chamber A with a crucible B therein having a 85 cover C, all these parts being shown in section. A layer D is shown in the bottom of the crucible representing zinc oxid or ore mixed with or covered by charcoal E, to act as the reducing agent. The mineral or carbon is preferably reduced to a divided state.

Ingots of copper F are shown resting upon the charcoal E, and when the crucible is heated to the proper temperature the charcoal combining with the oxygen of the 95 zinc oxid generates carbon-monoxid (CO), which is partly retained in the crucible by the cover C, and forms a reducing atmosphere therein which protects the alloy that is formed by the absorption of the vapor. 100

Burner-inlets J are shown in the walls of the furnace, and burners would be provided to heat the chamber.

The heat is regulated to volatilize the zinc at a temperature below that of melted 105 copper, and the vapor of the zinc is thus brought into contact with the heated surface of the copper ingots. The copper while thus heated absorbs the zinc vapor, which combines with the copper to form a film of 11

brass alloy upon the surface of the copper, the temperature in the crucible being sufficient to melt this alloy so that it runs off and accumulates in the bottom of the crucible.

5 The process of absorption is continuous, as the zinc vapor attacks the surface of the copper where it is exposed by the running off of the alloy, and the formation of such alloy upon the surface of the copper continues as long as the zinc vapor is supplied, with the effect of converting the copper and zinc vapor into the alloy desired.

10 The proportions of the two metals in the alloy depends upon the proportions placed in the crucible, as the zinc vapor is almost wholly utilized by union with the copper.

15 It will be understood from the above description that the operation practised with the ingredients all in one crucible does not consist in merely melting the ingredients together, or subjecting them to the melting temperature of copper, but that the temperature is intentionally maintained below that of melted copper, so as to economize in 20 the fuel and prevent any diffusion or loss of the zinc vapor. When heating all the ingredients in one crucible the copper is separated from the zinc oxid or ore, and is kept apart from the alloy, as formed, so as to 25 maintain a continuous exposure of the copper's surface to the zinc vapor.

30 Where circumstances permit or require it, the zinc vapor may be generated in a chamber or furnace separate from that in which the copper is heated, with provision to convey the metallic vapor from the point of generation to the point of alloying with the copper.

35 Fig. 2 shows a furnace for operating in such manner, the furnace being provided with chambers *a* and *a'* connected by a passage *a\**, in which chambers the zinc and copper respectively would be heated, the tap-hole *g* being closed during the alloying operation, and the copper being heated in the chamber *a'* to an alloying temperature while the zinc is heated in the chamber *a* to a vaporizing temperature, so that its vapor passes through the passage *a\** into the 40 chamber *a'*, where it is absorbed by the copper.

45 Inlets *b* are shown over the chambers to insert the metal thereat, such inlets being closed by covers *c* provided with lifting-bails *d*. A spout *f* is shown connected with the tap-hole *g*, by which the alloy may be withdrawn from the furnace at the close of the alloying operation.

50 From the above description it will be understood that the more fusible metal may be vaporized in any convenient manner, so as to be absorbed by the less fusible metal heated to a suitable temperature.

55 My invention does not consist in the mere melting of zinc and copper together, or the

mere heating of zinc ore and copper to form an alloy, but consists in subjecting the copper to the vapor of the alloying metal and producing a molten alloy of the two metals.

60 This invention permits the copper to be alloyed with the more fusible metal without melting the copper, and also in one form of the invention it permits the melting of the copper in one chamber or furnace and 65 the vaporizing of the zinc in another chamber or furnace, as stated above, and conducting the vapor into the chamber where the copper is heated, to form the alloy therein.

70 Where the zinc and copper are heated in the same receptacle, the copper is carefully separated from the zinc ore to prevent its immersion in the molten alloy, which would prevent the access of the vapor to the surface of the copper, and the continuous formation of the alloy in a molten state, as desired.

75 This separation is effected by placing the alloying element in the bottom of the receptacle and placing a layer of porous material like the charcoal *E* upon the top of the said element, thus supporting the copper above the level of the alloy.

80 After the charcoal is consumed the copper is prevented from contact with the molten alloy by the layer of earthy material, which remains after the zinc is extracted from the ore. Such earthy material prevents immersion of the copper in the alloy during the formation of the latter. The 85 surface of the copper is thus exposed continuously during the alloying operation to the vapor of the zinc.

85 What I do claim as my invention, and desire to secure by Letters Patent is:

90 1. The process of alloying copper with a more fusible metal, as zinc, lead, &c., which consists in heating the copper and the alloying metal free from contact with one another, the copper being heated to an alloying temperature and the zinc to at least a vaporizing temperature, and subjecting the copper thus heated to the vapor of the zinc until the desired alloy is formed in a molten state.

95 2. The process of alloying copper with more fusible metals as zinc, lead, &c., which consists in heating the copper in one chamber or receptacle to an alloying temperature, vaporizing the alloying metal in another 100 chamber, and conveying the said vapor into contact with the heated copper and forming an alloy of the said metals in a molten state.

105 3. The process of alloying copper with more fusible metals, as zinc, lead, &c., which consists in melting the copper in one chamber, vaporizing the alloying metal in another chamber, and conveying the said vapor into contact with the melted copper and 110

forming an alloy of the said metals in a molten state.

4. The process of alloying copper with more fusible metals as zinc, lead, &c., which consists in melting the copper in one receptacle, reducing an oxid or ore of the alloying metal in a separate chamber and

regenerating a vapor of the alloying metal, conveying the said vapor into contact with the molten copper, and forming an alloy of 10 the said metals in a molten state.

In testimony whereof I have hereunto set my hand.

HILLIARY ELDRIDGE.